

## UNITED STATES PATENT OFFICE

ROBERT C. MORAN, OF WOODBURY, NEW JERSEY, ASSIGNOR TO VACUUM OIL COMPANY, OF NEW YORK, N. Y., A CORPORATION OF NEW YORK

## LUBRICATING OILS

No Drawing.

Application filed August 16, 1929. Serial No. 386,489.

- The present invention relates to improvements in compounded lubricating oils.
- It is well known that the lubricating qualities of mineral oils may be improved by the addition of fatty acids, either alone or as constituents of vegetable or animal fats. The most commonly used fatty acids for improving the lubricating property of mineral hydrocarbon oils are oleic and stearic acids.
- 10 The use of these fatty acids involves certain disadvantages. Oleic acid is liquid at ordinary temperatures and hence does not adversely affect the pour test of lubricating oils when mixed therewith, but, due to its 15 unsaturated character, oleic acid readily oxidizes so that mixtures thereof with lubricating oils are decidedly objectionable in practice because of their tendency to sludge formation and the development of corrosive 20 acidity. Stearic acid, on the other hand, is a saturated acid and hence is free from that objection to oleic acid of imparting to its mixtures with lubricating oils the ready 25 tendency to sludge formation and the development of particularly corrosive acidity. But stearic acid is objectionable in its effect 30 on the pour test of lubricating oils when admixed therewith. For instance, a lubricating oil having a pour test of  $-5^{\circ}$  F. showed, after the addition of 2% stearic acid, a pour test of  $+36^{\circ}$  F.
- The present invention resides in the discovery that the addition, to a mineral oil, of the acid product of the interaction of oleic 35 acid and benzene in the presence of aluminum chloride, will give to the mineral oil a lubricating quality similar to that obtained by the addition of saponifiable oils and fats to mineral oils.
- 40 The acid may be prepared in the following manner. To 200 gms. of oleic acid dissolved in 400 gms. of dry benzene are added 100 gms. (1.2 molecular proportions) of coarsely powdered aluminum chloride.
- 45 When the reaction has moderated, the mixture is gently heated (finally to  $80^{\circ}$  C.) with occasional shaking, until hydrochloric acid is no longer evolved. The heating requires about six hours. The mixture is then poured 50 into 600 c. c. of 20% hydrochloric acid, and

the benzene removed by steam distillation. The residual brown, viscous oil may be used as such, but preferably is fractionated under reduced pressure, the distillate being finally obtained as a yellowish oil, boiling point 55 about  $250^{\circ}$  C. at 4 m. m., and solidifying at about  $15^{\circ}$  C. The crude or redistilled product is particularly suitable for use in improving the lubricating effectiveness of lubricating hydrocarbon oils, as it is a liquid, 60 readily miscible with said lubricating oils and is essentially of a saturated character. Hence, when admixed with lubricating oils, it has no adverse effect on the pour test such as is caused by stearic acid, nor does it 65 impart to the mixture the tendency to sludge formation and the corrosive acidity characteristic of oleic acid.

As an illustration of this invention, a lubricating oil having a specific gravity of 0.90 70 was mixed with 3% of acid without adverse effect on the pour test. The mixture, atomized with air at about  $300^{\circ}$  F. and the atomized stream directed upon a test piece of Admiralty metal, maintained at about room temperature, resulted in no corrosion of the metal 75 after about ten days. Upon similar test conditions, a 3% addition of oleic acid to the same lubricating oil gave a mixture which corroded the Admiralty metal in a relatively rapid manner.

Usually the acid is added to the body of hydrocarbon lubricant in amounts of from approximately 0.5% to approximately 3% of the volume of the latter. The addition of 85 these amounts of the acid, while greatly improving the lubricating properties of the oil, with corresponding lowering of the interfacial tension against water, has no effect upon the original pour test of the oil. The 90 importance of this feature with respect to cold weather lubrication is obvious.

While there has been specified 3% of acid in the above lubricating oil mixture for illustrative purposes, lesser and greater quantities of the acid may be used with advantage in certain cases.

The acid produced by the process herein described is a phenyl-stearic acid of which the precise constitution is not known. As it 100

was first described by Nicolet and de Milt it may be designated as "Nicolet and de Milt's acid". Its theoretical formula is believed to be either



or



- 10 or it may contain both of these isomers. So far as known, either or both of these isomers may be used with equal effectiveness.

What I claim as my invention and desire to secure by Letters Patent is:

15. A lubricant consisting chiefly of mineral lubricating oil, with the addition of a relatively small amount of Nicolet and de Milt's acid.

ROBERT C. MORAN.

20

25

30

35

40

1

50

5

1